

## UNITED STATES PATENT OFFICE

2,168,107

## CONTAINER STRUCTURE WITH INHIBITOR

Arthur E. Stevenson and Sylvester L. Flugge,  
Chicago, Ill., assignors to Continental Can Com-  
pany, Inc., New York, N. Y., a corporation of  
New York

No Drawing. Application April 19, 1935, Serial  
No. 17,357. Renewed April 18, 1939

4 Claims. (Cl. 99—181)

This invention relates to improvements in containers for food products, and is particularly concerned with the provision of a container which is capable of enclosing a food product of corrosive character, i. e., one which normally tends to attack tin plate or like product normally employed in making at least a portion of the container.

According to the present invention, the food product is prevented from attacking the corrodible portion of the container by contacting this food product with a substance which operates upon contact with the food product to inhibit such corrosion.

15 A particularly advantageous manner of introducing and maintaining the substance is to include it as an ingredient in a coating, such as the sealing compound which is employed for establishing the hermetic seal of the container. It is customary in closing tin cans, for illustration, to make the final seal by crimping or seaming the edges of the cover and body portions of the container into interlocking relation with one another; the hermeticity of the seal being maintained by providing a plastic seal at this junction. One manner of providing the seal is to form the cover with a peripheral groove, and to distribute a plastic sealing compound into this groove and permit it to become semi-solid or solid therein and adherent to the groove walls. When the cover is located upon the end of a container body, and crimped thereto, this sealing compound is placed under compression and thus serves to form and maintain the tight sealing desired.

35 When corrosive substances, such as the juices of certain preserved fruits, come into contact with tin plate or like material, they tend to attack this material, particularly if the plating is imperfect, and to cause perforations of the containers; and also, when such material is dissolved, the true color of the food product is affected deleteriously.

According to the present invention, the corrosive action is inhibited by presenting to the food product a substance which tends to prevent this attack, this substance being preferably introduced as a component of a coating, particularly as a component of the sealing material, and in proportion from five to twenty percent by weight of the "dry solids" of the coating.

50 The preferred substances for this purpose are compounds containing carbon, sulphur and nitrogen, three particular types being found highly advantageous. These types are: (1) thio-urea and substituted thio-ureas such as allyl thio-urea; (2) sulphur-containing amino acids such

as cystine, cysteine and methionine; and (3) sulpho-cyanates, particularly the alkali sulpho-cyanates such as potassium, sodium and ammonium sulpho-cyanates. These materials are innocuous in the quantities used (e. g., 2 to 4 5 milligrams are available to the can contents for a No. 2 can) and of themselves produce no fundamental change in the food product in the quantity utilized and brought into contact with the food product. Such materials may readily be incorporated in the sealing compounds normally employed in the manufacture of cans and like containers, and in the quantities utilized, they produce no disadvantageous effect upon the consistency of the sealing compound mixture itself. 10

For example, in the canning of sour cherries, a sealing composition of resinous or rubber base may have ten percent of thio-urea incorporated therewith, in proportion by weight relative to the deposited materials (i. e., the "dry solids") left 20 upon evaporation of solvents and dispersing agents present.

Other compositions of the nature set forth and claimed herein may be employed in proportions which may be varied according to the 25 particular material utilized, the particular food product being preserved, and the nature of the corrodible container structure, and the relative proportion thereof with respect to the volume of the food product.

What is claimed, is:

1. A sheet metal container of tin plate for food products, of corrosive character comprising a body portion, ends seamed to the body portion, and a plastic sealing compound within the seams for hermetically sealing the container, said sealing compound being exposed to the food product contained in the container and including a base effective for sealing and having a substance uniformly admixed therewith which operates upon 35 contact with the food product to inhibit the corrosion thereby upon said tin plate, said substance being one of the carbon, sulphur and nitrogen containing compounds consisting of thio-urea, allyl thio-urea, cystine, cysteine, methionine and alkali sulpho-cyanates. 40

2. A container structure as in claim 1 in which the inhibitor substance comprises thio-urea.

3. A container structure as in claim 1 in which the inhibitor substance comprises cystine. 50

4. A container structure as in claim 1 in which the inhibitor substance comprises alkali sulpho-cyanates.

ARTHUR E. STEVENSON.  
SYLVESTER L. FLUGGE. 55